

# UNITED STATES PATENT OFFICE.

HERMAN L. HARTENSTEIN, OF CONSTANTINE, MICHIGAN, ASSIGNEE, BY MESNE ASSIGNMENTS, TO CONTINENTAL INVESTMENT COMPANY, OF DULUTH, MINNESOTA, A CORPORATION OF MINNESOTA.

## MANUFACTURE OF CARBID.

No. 889,124.

Specification of Letters Patent.

Patented May 26, 1908.

Original application filed February 13, 1907, Serial No. 357,140. Divided and this application filed July 17, 1907.  
Serial No. 384,235.

*To all whom it may concern:*

Be it known that I, HERMAN L. HARTENSTEIN, a citizen of the United States, residing at Constantine, in the county of St. Joseph and State of Michigan, have invented certain new and useful Improvements in the Manufacture of Carbid, of which the following is a full, clear, and exact specification.

This invention relates more particularly to the manufacture of calcium carbide from limestone or lime and a carbonaceous material such as coal, etc., and it has for its primary object a method in which all of the advantages of the use of coal may be secured without any of the disadvantages of such element, such as excessive smoke generated in the furnace during the reduction operation, and the higher or excessive voltage required by reason of the presence of the particles of hard coal in the charge being treated or reduced.

Another object of the invention is to provide an improved method for the manufacture of carbid in which the small particles of lime or limestone will be bound into intimate association with the small particles of carbonaceous material during the reduction of the same in the electric furnace.

In carrying out the invention, I employ lime and carbonaceous material in the usual or any suitable proportions as heretofore practiced in this art and the lime is obtained in the usual or any suitable way but preferably by calcining limestone which has been previously pulverized or comminuted. The lime or calcined limestone is taken from the pre-heater or calcining furnace while in its highly heated condition and is mixed with the proper proportion of carbonaceous matter which, according to this invention, consists of a mixture of hard coal (anthracite coal) and coke; or charcoal. I preferably employ anthracite coal screenings, which are in a more or less fine or comminuted condition and to eighty or ninety per cent. of which I add from ten to twenty per cent. of the coke or charcoal, which is also previously ground or powdered. By using anthracite coal and coke it is practicable to utilize the cheaper grades of coke as, for example, breeze or refuse which is higher in ash and impurities than lump coke and contains much more than the anthracite coal. These two ingre-

dients are intimately commingled and mixed with the fine or pulverized lime or limestone while the latter is in its highly heated condition and the mass is then subjected to the action of the electric current in an electric furnace until reduced to a bath according to the established practice of this art. The anthracite coal is rich in carbonaceous material but its use is attended by objectionable results, such as excessive smoke which precludes a fair view of the electrodes when the furnace is opened for examination by the attendant from time to time during the operation and, moreover, it furnishes a high resistance to the current and as a consequence requires a higher voltage. These objections however, are sufficiently overcome by the addition of the percentage of coke or charcoal which adds greatly to the conductivity of the charge between the electrodes.

The result may be still further improved and facilitated by the addition to the carbonaceous constituent of a small percentage (say from three to twenty per cent.) of bituminous coal, rich in tarry compounds, say about five per cent. This, also, is employed in a state of fine sub-division and it is mixed with the lime or calcined limestone while the latter is in its highly heated condition after coming from the pre-heater or calcining furnace and by thus intermingling the bituminous coal with the lime or calcined limestone while the latter is hot it is converted into coke and its tarry constituent is more or less liquefied or softened and deposits itself upon the particles of calcined limestone as well as upon the particles of coke and anthracite coal and acts as a binder to hold these constituents of the carbonaceous material into intimate association with the lime, thereby giving every particle of lime its appropriate percentage of carbonaceous material and resulting in a final product which presents a degree of uniform reduction greater than that heretofore secured.

The soft coal may also be mixed with the anthracite or coke before being placed in the mixer with the highly heated limestone.

The temperature is sufficiently high to convert the tar and carbon of the coal into coke, and previous to or during the process of mixing it serves to act as a "binder" for holding together the coke, anthracite and highly

heated limestone of the charged mixture, while the soft coal is likewise converted into a coke and becomes a portion of the charge mixture when it leaves the mixer and is 5 placed in the electric furnaces.

It is understood that the particles of hot limestone and coke and anthracite coal become more or less mechanically united while the tarry matter of the soft coal is being expelled therefrom and converted into coke.

The volatile matter or gases that are expelled during the mixing process furnish heat elements, and at the same time materially aid the mechanical mixing process, by reason 15 of the boiling or agitation caused by the volatile matter of the soft coal in the presence of heat.

The gases produced by the addition of soft coal are also ample to prevent the admission 20 of air into the mixture and thereby prevent any possible oxidation of other carbonaceous

material (anthracite or coke) which is low in volatile matter.

The process herein described forms the subject matter of the claims of my application Serial No. 357,140, filed February 13th, 1907. 25

Having thus described my invention, what I claim as new therein and desire to secure by Letters Patent is—

A composition of matter for use in the manufacture of carbid, consisting of lime, bituminous coal, coke or charcoal and anthracite coal. 30

In testimony whereof I have signed my name to this specification, in the presence of two subscribing witnesses, on this eighth day of July A. D. 1907. 35

HERMAN L. HARTENSTEIN.

Witnesses:

H. E. SMITH,  
Wm. H. BROWNRIGG.